

Dec. 31, 1929.

W. H. KOBBE

1,741,522

SULPHUR CONTAINING COVERING

Original Filed Aug. 13, 1926

*Fig. 1.*



*Fig. 2.*



INVENTOR

William H. Kobbe

BY

Pennie, Davis, Marvin and Edmonds

ATTORNEY.

## UNITED STATES PATENT OFFICE

WILLIAM HOFFMAN KOBBE, OF NEW YORK, N. Y., ASSIGNOR TO TEXAS GULF SULPHUR COMPANY, OF BAY CITY, TEXAS, A CORPORATION OF TEXAS

## SULPHUR-CONTAINING COVERING

Original application filed August 13, 1926, Serial No. 129,086. Divided and this application filed April 12, 1928. Serial No. 269,488.

This invention relates to coverings made of fabric and has for its object the provision of certain improvements in the method of making coverings in part at least of fabric. More particularly the invention aims to provide an improved method of making coverings comprising a fabric impregnated with molten sulphur. This application is a continuation of my copending application, Serial No. 129,086.

The invention is based on my discovery that the association of sulphur with fabric coverings, preferably by impregnation of the fabrics with sulphur, imparts to the fabric such a degree of strength and/or rigidity as to render it admirably adapted for making coverings for numerous rigid articles. The association of sulphur with fabrics, preferably by impregnation of the fabrics with sulphur, furthermore provides an intimate contact between the article covered and the sulphur impregnated fabric, through the contraction of the sulphur upon cooling and crystallization. The invention thus contemplates the provision of new articles of manufacture in the nature of coverings made in whole or in part of sulphur containing or sulphur impregnated fabric, and methods of making the same.

By "fabric" I mean to include any pliable fibrous material, such as the various textiles, felts and other cloth-like materials, made of either organic or inorganic fiber. In particular, I mean to include fabrics made from asbestos or other mineral, fibers made of wool, silk, cotton, hair, jute, hemp, flax, wood pulp and other animal and vegetable fibres. More especially, I mean to include burlap, canvas, cotton, flannel, all types of felt and in fact all classes of fabrics and/or textile products.

In carrying out the present invention, I treat the fabric with sulphur so as to effect an association with the fabric of an appropriate amount of sulphur in such as to impart to the fabric a desired degree of strength or rigidity. The desired association between the fabric and sulphur may be brought about in various ways, as for example, by impregnating the fabric with sulphur through immersion of the fabric in molten sulphur. The association of the sulphur with the fabric may also be accomplished by passing the fabric over rolls carrying molten sulphur, as well as by including solid sulphur in the fabric in any appropriate way and subsequently fusing the sulphur in contact with the fabric by the application of heat.

Heretofore metallic pipe lines and other structures which are installed underground have been subjected to corrosive action. The corrosion of metal pipe lines in particular is a very serious problem especially in certain soils containing salts or other active chemicals. This is notably the case in the oil fields of the southwestern portion of the United States and portions of California. In some cases the rapid corrosion of the pipe lines necessitates the removal or repair of these lines within two years and even within a shorter period. Destruction by saline waters of oil well tubing is also very common in the same districts.

Elemental sulphur is chemically very resistant to the action of most reagents, it is impervious to water, and in many other respects is suited for protective purposes when applied to articles which are exposed to any of these reagents. The brittleness of elemental sulphur alone makes it very difficult to apply to large unbroken surfaces, and also makes materials covered in this manner very difficult to handle without rupturing the sulphur covering.

I have discovered a method of utilizing the protective qualities of sulphur as a covering for objects exposed to corrosion by associating the sulphur with a fabric. In accordance with the present invention, the article to be protected is covered with a fabric impregnated with molten sulphur in such a way that

the contraction of the sulphur upon crystallizing causes the sulphur impregnated fabric to adhere closely to the article covered. The following is an illustration of the protective covering of the invention as applied to a metal pipe:

A porous material in the nature of a fabric capable of absorbing a high percentage of molten sulphur is cut into strips of any appropriate width. The porous material, preferably a fabric, is then thoroughly saturated by passing it through a bath of molten sulphur. The impregnated fabric upon withdrawal from the bath and while the sulphur is still hot and molten, is then applied to a revolving length of pipe or other similar material to be protected. The material on emerging from the bath of molten sulphur may be wound upon the pipe, either straight or spirally, or in any similar appropriate manner until a sufficient thickness of material is applied to the pipe. The thickness of the protective coating applied to the pipe or article being covered may be of any desired amount depending upon the type of material and the condition of handling and service. For pipe covering, I have found a thickness of substantially one quarter of an inch sufficient to give satisfactory service, but this thickness may be increased or diminished so as to meet any given requirement. The molten sulphur as it contracts with the pipe attaches itself thereto and each succeeding layer of the sulphur impregnated fabric is closely welded to the layer next below it by the molten sulphur absorbed within the fabric and adhering to the surface thereof.

When a sufficient number of such layers are applied, the pipe with its covering of sulphur impregnated fabric is permitted to cool. In cooling the absorbed sulphur solidifies by crystallization with resulting contraction. This contraction not only binds the mass tightly to the enclosed pipe, but results in a homogeneous monolithic stone-like covering.

In practicing the invention various textiles or fabrics are best suited for this purpose because of their tensile strength and high degree of absorption, but I prefer to use cotton flannel, felt or similar material. The strips may be of any width so as to admit of application by wrapping spirally and obtaining thereby a uniformly smooth covering. When spiral wrapping is employed, a strip of from 5 to 6 inches wide is sufficient, but in some cases a wider strip may be used depending upon the resiliency of the material and its ability to conform to the spiral wrappings.

A length of six inch line pipe, for example, approximately 20 feet long, is slowly revolved by mechanical means in a horizontal position while a strip of sulphur impregnated cotton flannel or other fabric is applied to the pipe. Before the cotton flannel is applied to the pipe it passes through a bath of molten sul-

phur at a temperature of approximately 150° C. This sulphur bath may be in the form of a trough or small tank of appropriate size, the fabric passing in at one end, carried under the surface of the molten sulphur on appropriate rolls or other mechanical means, and applied to the revolving pipe upon which the impregnated material is being wound. Such a strip of fabric is not only fully saturated with sulphur by its immersion in the bath, but it leaves the bath and is wound on the pipe in a dripping condition, the temperature being such that solidification does not take place until the fabric has passed around the pipe and for an appreciable time thereafter. The subsequent plies are superimposed upon the preceding layer of this sulphurized fabric in the same manner, and in this way I build up a protective covering of any desired thickness by applying as many layers as may be necessary. In most cases four plies of the sulphurized fabric are sufficient to give adequate protection.

The molten sulphur crystallizes after the covering has been applied as described. The crystallization takes place not only within the fabric but between the plies thereof and at the same time increases in density which results in a marked shrinkage. This shrinkage takes place not only when the liquid sulphur passes to the monoclinic stage of crystallization but again as this monoclinic sulphur gradually changes to the stable rhombic condition. In other words, the final and permanent state of the sulphur is materially less in mass than that of the molten material originally applied, and this action is largely responsible for the great strength, homogeneity and imperviousness of the finished covering. Such a covering may consist of from 75 to 95% of sulphur by weight, depending upon the porosity of the material used and the quantity of excess sulphur thereon when applied to the pipe. This results in what is in fact a monolithic or stone-like covering bonded not only to the pipe surface but each layer bonded to the adjacent layer with no indication of separate and distinct layers. This sulphur impregnated fabric covering is extremely tough, and can only be removed from the pipe by resorting to such means as a cold chisel or some similar cutting and wedging operation, or by means of the application of sufficient heat to melt the crystallized sulphur.

In Fig. 1 of the drawing I have illustrated a metal pipe covered with the sulphur impregnated fabric of the invention. The pipe is cut away so as to better illustrate the pipe and the nature of the covering.

Fig. 2 of the drawing is a sectional view showing the manner of applying the impregnated fabric covering of the invention to the thread and coupling ends of a metal pipe.

In the drawing a metallic pipe 5 is cov-

ered with the monolithic sulphur impregnated covering 6 of the invention. The contraction of the sulphur upon crystallizing causes the covering 6 to draw tightly about the exterior of the pipe 5 from all sides with equal force, so that the bond between the pipe 5 and the covering 6 is made infinitely tight and the whole mass of the covering 6 is bound by the force of crystallization into a monolithic or stone-like structure by the shrinkage of the crystallized sulphur. The layers of the covering 6 are wound on the pipe 5 spirally. The joints 7 where the spiral wrappings join each other are visible on the surface of the covering 6, but are bound or cemented firmly by congealed sulphur.

The fibrous nature of the fabric used in the covering 6 binds the brittle or frangible particles of sulphur together in such a manner that the covering assumes not only a rigid form but a tough structure as well. The shrinkage of the covering material brought about by crystallization causes the whole mass to assume such a dense form that the various layers of which the covering is built are thoroughly merged into one another and are not visible when the covering is broken or cut as shown in the drawings.

In Fig. 2 of the drawing when covering pipes which have threaded connections for attaching one length of the pipe to the next adjoining length, I prefer to screw a coupling 10 securely to one end of the pipe 5 before covering it with the sulphur impregnated fabric 6. The threads 8 at the opposite end of the pipe may be appropriately protected before the sulphur impregnated fabric is applied. The sulphur impregnated fabric 6 is then applied to the pipe from the extreme end 14 of the attached coupling 10 and is terminated at the point 9 where the pipe threads begin near the opposite end of the pipe; thus these threads 8 are left exposed. When one covered pipe is screwed into the next covered pipe, the exposed threads 8 are almost entirely covered by the coupling 10 of the adjoining pipe and the protective covering of one pipe approaches very closely the protective covering of the next adjoining pipe. The short intervening space between the coverings is then wound manually with sulphur impregnated fabric of the same, or like nature as the material which was used for the protective covering 6. The molten sulphur of this manually applied strip melts a sufficient portion of the sulphur in the already sulphur impregnated covering so that a permanent bond is made between the newly applied material and the covering already on the pipes.

Bolted, flanged or riveted pipe joints are not covered with the protective covering until after the coated lengths of pipe are jointed together. The joints are then covered manually by means of sulphur impregnated strips

of fabric in the same manner as was used in filling the gap when threaded pipes are joined.

I do not intend to confine myself entirely to the method of operation described in the example given herein. This method may be varied in many details without departing from the spirit of the invention. Thus, for example, a pipe or other structure may be straight wound rather than spirally. This necessitates strips preferably as wide as the length of the pipe or other structure which is being covered.

The pipe, or other structure, on the other hand, may be wrapped with the requisite number of plies of fabric and then immersed as a whole in the saturating bath. This procedure, however, is not economical and is wasteful of heat for by this method it is necessary to raise the metal of the structure being covered to the temperature of the bath before impregnation can be fully brought about, and the whole mass must be then subjected to cooling upon its removal from the bath before complete crystallization can take place.

I prefer to use elemental sulphur as the impregnating means for the fabric, but it is sometimes desirable, for various reasons to add an inert filler to the sulphur, in order to produce a sulphur composition possessing greater strength and/or resistance than can be obtained by sulphur alone. An inert filler of this nature having a specific gravity approximating that of sulphur and in a finely ground state, maybe suspended in the impregnating bath approximately in equal parts by weight. The fabric passing through a bath made up in this manner carries the mixture of filler and sulphur along with it and although it may penetrate the fabric only in part, it adheres to the surface of the fabric and produces a pipe covering of great strength, imperviousness and tenacity. It will be understood that the invention is not limited to pipe coverings although particularly efficacious and applicable for this purpose, but may be used on a great variety of other materials, such, for instance, as guy rods, especially the portion submerged beneath the surface of the ground or at the ground line or oil well tubing or wherever metal is attacked and destroyed by corrosive or other destructive agencies.

I claim:

1. The method of making articles having coverings composed in part at least of sulphur-impregnated fabric, which comprises impregnating fabric in a bath of molten sulphur at a temperature of substantially 150° C., wrapping the hot, sulphur-impregnated fabric upon the article to be covered, causing the temperature of the sulphur-impregnated fabric to be lowered and the sulphur to contract and solidify in crystalline form within the interstices of the fabric.

2. An article having a protective covering firmly attached thereto, said covering comprising a fabric having its interstices filled with crystalline sulphur.
- 5 3. An article having a protective covering firmly attached thereto, said covering comprising a monolithic sulphur-impregnated fabric containing from 75% to 95% of sulphur.
- 10 4. An article having a protective covering firmly attached thereto, said covering comprising a monolithic sulphur-impregnated fabric.

In testimony whereof I affix my signature.

15 **WILLIAM HOFFMAN KOBBE.**

20

25

30

35

40

45

50

55

60

65